

## UNITED STATES PATENT OFFICE

2,648,602

## HIGH STRENGTH STEEL FOR HIGH-TEMPERATURE SERVICE

Peter Payson, New York, and Joe Gin-Young Chow, Long Island City, N. Y., assignors to Crucible Steel Company of America, New York, N. Y., a corporation of New Jersey

No Drawing. Application January 17, 1952,  
Serial No. 267,003

3 Claims. (Cl. 75—126)

1

This invention relates in general to a forgeable alloy steel for service under high stress at temperatures around 1100° F. for such parts for example, as bolts, studs, flanges and turbine blades in the modern steam power plants and for wheels in gas turbines. It is desirable that such parts have high strength both at room and elevated temperatures.

Although some alloy steels containing appreciable amounts of nickel, cobalt, or columbium have been proposed for such applications, the present scarcity of these metals makes it desirable that a steel be available which has adequate strength and oxidation resistance for service at temperatures up to about 1100° F., and yet be as free as possible of these strategic elements.

It is the object of this invention to provide a forgeable alloy steel, which is heat treatable to high strength levels; which is adequately resistant to oxidation under long time exposure to temperatures of about 1100° F.; which has high strength at these temperatures; and which neither requires nor employs any of the strategically critical elements, nickel, cobalt and columbium.

The steel of the present invention contains as essential alloying additions, chromium, tungsten, molybdenum, vanadium and manganese, with chromium as the major addition, i. e. about 11 to 14%, together with relatively small amounts of the remaining elements mentioned, as brought out more specifically below.

To provide adequate resistance to oxidation we use a minimum of about 11% chromium in our steel and we may use as much as 14%. With higher contents of chromium it is difficult to develop high strength in the steel because of the marked tendency of chromium to inhibit austenite formation, and without such formation, it is not possible to form strength-giving martensite in the steel by heat treatment.

To give the steel strength at elevated temperatures, we use the active carbide forming elements vanadium, tungsten, and molybdenum in combination in relatively small amounts, namely from about 0.20 to .70% vanadium; from about 1.0 to 2.5% tungsten; and from about 1.5 to 4.0% molybdenum. As is well known, these elements in steel cause resistance to softening over the range of temperature from about 900 to 1100° F., and hence provide strength in the steel at these temperatures. The molybdenum content is preferably kept higher than the tungsten content.

2

Although it has been maintained that tungsten and molybdenum are interchangeable in the ratio of one part tungsten for about 0.6 part molybdenum (see Gill et al., "Tool Steels," ASM, 1944, page 510), we have found, as will be shown below, that the combination of both tungsten and molybdenum in our steel imparts higher elevated temperature strength, than is obtainable with just one in sufficient amount to make up for the other.

Since chromium, vanadium, tungsten, and molybdenum, all are "ferrite formers," that is, they tend to inhibit the formation of austenite in the steel, and hence make the steel non-hardenable by ordinary heat treatment, it is necessary to provide in the steel of our invention, compensating "austenite formers," viz. carbon and manganese. We find that about .20% carbon along with about 0.50% manganese are sufficient to provide at least 75% austenite in the steel at about 2000° F. when the other elements are present in the amounts mentioned. More than 10% residual ferrite is detrimental to the strength of the steel. We find it desirable to limit the carbon to about .40%, and the manganese to about 1.5% on the high side, in order to avoid retention of austenite in the heat treated steel, and to provide adequate ductility in the steel at room temperature after heat treatment.

The silicon in the steel should be sufficient to assure thorough deoxidation, i. e. on the low side from an effective amount of about 0.1%. And generally we limit the silicon to about 0.5% on the high side, since silicon is also an active ferrite former.

The broad and preferred ranges of analysis of our steel are as follows:

|    | Analysis, Percent |           |
|----|-------------------|-----------|
|    | Broad             | Preferred |
| C  | 0.20/0.40         | 0.25/0.30 |
| Mn | 0.50/1.50         | 0.60/0.90 |
| Si | up to 0.5         | 0.15/0.40 |
| Cr | 11.0/14.0         | 12.0/13.0 |
| V  | 0.2/0.70          | 0.3/0.5   |
| W  | 1.0/2.5           | 1.5/2.0   |
| Mo | 1.5/4.0           | 2.0/2.5   |
| Fe | Remainder         | Remainder |

In order to secure the full effect of the alloying elements in the steel for high strength at elevated temperatures, we heat treat with a minimum austenitizing temperature of 1900° F., and we preferably use 2000° F. The steel is then

either oil quenched or air cooled (if the section is relatively small) to room temperature, and then tempered at 1200° to 1300° F., the lower temperature being preferred where the service temperature does not exceed 1100° F. The mechanical properties attainable at room temperature after heat treatment are shown in Table I.

TABLE I  
*Room temperature mechanical properties of steel of this invention.*

[Test pieces quenched in oil from 2000° F. and tempered at 1200° or 1300° F., for 2 hours.]

| Bar  | C   | Mn  | Si  | Cr    | V   | W    | Mo   |
|------|-----|-----|-----|-------|-----|------|------|
| 3640 | .27 | .80 | .29 | 12.64 | .41 | 1.75 | 2.30 |
| 3642 | .34 | .74 | .26 | 12.60 | .38 | 1.74 | 2.30 |

  

| Bar  | Tempered at | Rockwell "C" | Tensile Strength, p. s. i. | 0.2% Yield, p. s. i. | E1. in 1.4-in. percent | Red Area, percent |
|------|-------------|--------------|----------------------------|----------------------|------------------------|-------------------|
| 3640 | 1200° F.    | 39.5         | 180,000                    | 140,000              | 16.6                   | 47                |
| 3640 | 1300° F.    | 36.5         | 164,000                    | 128,000              | 15.9                   | 38                |
| 3642 | 1200° F.    | 42.5         | 191,000                    | 148,000              | 14.7                   | 36                |
| 3642 | 1300° F.    | 38           | 169,000                    | 132,000              | 14.7                   | 40                |

After such heat treatment these steels can withstand a stress of about 50,000 p. s. i. for 1000 hours at 1100° F., which is a higher value than is attainable in any known steel free from appreciable amounts of nickel, cobalt, and columbium, and is superior to some steels which contain these elements; for example, the 5% cobalt steel of U. S. 2,462,665; and the austenitic 18 Cr-8 Ni steels; Types 302, 347, and 316.

Data showing the effect on the heat treatable 12% Cr steel of various amounts of tungsten and molybdenum on the time to rupture under stress at 1100° F., are shown in Table II.

TABLE II

*Stress-rupture values at 1100° F.*

[Samples oil quenched from 2000° F., and tempered at 1200° F. for 2 hours, then stressed as indicated.]

| Bar  | Analysis, Percent |     |     |       |     |      |      | "Equivalent Mo" <sup>1</sup> | Time to Rupture, hours |                 |
|------|-------------------|-----|-----|-------|-----|------|------|------------------------------|------------------------|-----------------|
|      | C                 | Mn  | Si  | Cr    | V   | W    | Mo   |                              | 62,000 p. s. i.        | 56,000 p. s. i. |
| 3633 | .28               | .74 | .29 | 12.47 | .38 |      | 2.30 | 2.3                          | 6                      | -----           |
| 3636 | .27               | .70 | .27 | 12.37 | .37 | .75  | 1.30 | 1.8                          | 15                     | 317             |
| 3635 | .27               | .60 | .26 | 12.32 | .38 |      | 3.29 | 3.3                          | 153                    | 334             |
| 3637 | .27               | .73 | .27 | 12.63 | .39 | .73  | 2.30 | 2.7                          | 128                    | 361             |
| 3641 | .34               | .75 | .25 | 12.58 | .41 | .75  | 2.37 | 2.8                          | 138                    | 469             |
| 3640 | .27               | .80 | .29 | 12.64 | .41 | 1.75 | 2.30 | 3.3                          | 167                    | 416             |
| 3642 | .34               | .74 | .26 | 12.60 | .38 | 1.74 | 2.30 | 3.3                          | 201                    | 416             |

<sup>1</sup> "Equivalent Mo" equals 0.6 X Percent W plus Percent Mo.

These data show that tungsten is not merely a substitute for molybdenum in the approximate amount of 1 part W to 0.6 part Mo, but acts independently to improve the stress rupture properties of the steel. Thus the W-bearing steel, Bar 3636, with "equivalent Mo" less than that of Bar 3633, is the better of the two. The W-bearing steels Bars 3637 and 3641, with "equivalent Mo" less than that of Bar 3635, are about equal to it in stress rupture properties at 1100° F.; and the W-bearing steels, Bars 3640 and 3642,

and 3642, with the same "equivalent Mo" as Bar 3635 are definitely superior to the latter.

The steel of the invention as ordinarily produced will contain from about .03 to 0.08% nitrogen, and may advantageously contain up to about 0.35% nitrogen, it being understood that the nitrogen can partially replace the carbon, to the extent that the carbon may be reduced to about 0.1%.

## 10. What we claim is:

1. A forgeable and heat treatable alloy steel which as heat treated possesses high strength and good ductility at room temperature, and high stress-rupture properties at temperatures up to about 1100° F., said steel having substantially the following composition: 0.2 to 0.4% carbon; 0.5 to 1.5% manganese; 11 to 14% chromium; 0.2 to 0.7% vanadium; 1 to 2.5% tungsten; 1.5 to 4% molybdenum; from an effective amount to about 0.5% silicon; remainder iron.

2. A forgeable and heat treatable alloy steel which as heat treated possesses high strength and good ductility at room temperature, and high stress-rupture properties at temperatures up to about 1100° F., said steel having substantially the following composition: 0.25 to 0.3% carbon; 0.6 to 0.9% manganese; 0.15 to 0.4% silicon; 12 to 13% chromium; 0.3 to 0.5% vanadium; 1.5 to 2% tungsten; 2 to 2.5% molybdenum; remainder iron.

3. A forgeable and heat treatable alloy steel which as heat treated possesses high strength and good ductility at room temperature, and high stress-rupture properties at temperatures up to about 1100° F., said steel having substantially the following composition: 0.1 to 0.4% carbon; 0.5 to 1.5% manganese; 11 to 14% chromium; 0.2 to 0.7% vanadium; 1 to 2.5% tungsten; 1.5 to 4% molybdenum; from an effective amount

60 to about 0.5% silicon; from an effective amount up to about 0.35% nitrogen, the remainder iron.

PETER PAYSON.  
JOE GIN-YOUNG CHOW.

## 65. References Cited in the file of this patent

## UNITED STATES PATENTS

| Number    | Name         | Date         |
|-----------|--------------|--------------|
| 2,513,935 | Harris       | July 4, 1950 |
| 2,590,835 | Kirby et al. | Apr. 1, 1952 |